

## UNITED STATES PATENT OFFICE

STANLEY M. NORWOOD, OF FLUSHING, NEW YORK, ASSIGNOR TO ELECTRO METALLURGICAL COMPANY, A CORPORATION OF WEST VIRGINIA

## PRODUCTION OF CASTINGS WITH COATINGS COMPOSED OF HIGH-CHROMIUM ALLOYS

No Drawing.

Application filed March 10, 1931. Serial No. 521,809.

The invention relates to the production of castings consisting of inner portions or base metal of iron or steel and high-chromium alloy coatings which are resistant to abrasion and corrosion. The alloy coatings may contain about 12% or more of chromium but they commonly contain about 20% to 40% of chromium. The castings are made by pouring iron or steel into a mold which is covered with ferrochromium powder on the part or parts which correspond to the part or parts of the casting to be coated. The invention relates especially to the production of such castings or portions of castings in which the base metal is small in cross section or volume.

Heretofore castings with high-chromium alloy surfaces have been made by pouring ferrous metal into molds which were lined with powdered high-carbon ferrochromium. The ferrochromium used for this purpose contained about 4% to 6% carbon, 0.5% to 2.0% silicon, and about 65% to 70% chromium. With this ferrochromium, sufficient alloying was obtained in casting large cross-sections and surfaces of small curvature to produce alloy coatings with proper thickness to give protection from oxidation or chemical action. The coating could not be chipped or scaled off and it would not separate from the core of cast metal when the body was bent or broken. When the castings had an edge or surface portion which was angular or had a great curvature, and consequently had a comparatively small cross section of base metal associated with the portion, the alloying was incomplete, and continuous alloy coatings with sufficient thickness to give the desired properties could not be formed.

The principal object of the invention is to provide means of producing smoothness in the alloy coatings and flowing of the alloy into angular corners of the molds.

Another object of the invention is to provide means of producing completely alloyed continuous coatings on portions of castings which have a great curvature.

Another object of the invention is to provide means of producing complete alloying on castings in which the core metal consists

of a comparatively small volume or cross-section of metal as compared to the area of the coating.

The following description of one embodiment of my invention is illustrative. Ferrochromium composed of about 69% chromium, 4% silicon, 5% carbon and the remainder substantially iron was powdered. The powder which passed through a number 20 sieve and was retained on a number 60 sieve was mixed with sodium silicate solution to make it adherent to the mold, and the walls of a mold were coated with a layer of the composition about one-sixteenth of an inch thick. The mold was adapted to produce a casting about two inches thick by four inches wide by eight inches long with rectangular faces. Thus the coatings along the sharp edges of the mold and around the solid angles at the corners of the mold were subjected directly to the influence of only a small volume or pencil of molten base metal when the base metal was poured. Carbon steel containing about 0.5% carbon was heated to casting temperature and cast into the mold. Upon cooling, it was found that all the corners and edges of the mold were completely filled and the base metal was completely covered with a uniform adherent coating of high-chromium alloy.

It has been found that the desired results can be obtained by the presence of three to seven percent of silicon in the ferrochromium alloy powders used for lining the mold. The ferrochromium may be varied from about 60% to 96% chromium, the remainder being iron with about 3% to 7% silicon and about 1% to 6% carbon. Excellent results are obtained when about 4% to 6% carbon is present. The silicon may be present as an alloy constituent of the ferrochromium alloy, or ferrosilicon powder may be mixed with ferrochromium powder to give a mixture of coating powder which contains the requisite proportion of chromium, carbon and silicon. The use of mixed ferrosilicon and ferrochromium powder has been found advantageous with base metals which can be cast at lower temperatures than the temperatures most suitable for the best results with high-carbon ferrochromium powders, for example

cast iron. The combination of powders has been found to aid in fusing together and alloying the base metal and the constituents of the powders. For this purpose I prefer to use ferrosilicon which contains about 50% to 60% silicon, but higher or lower silicon-containing alloys can be used.

It is necessary to size the powders used for this purpose in order to obtain sufficient penetration and alloying of the base metal with the high chromium powder to produce high chromium coatings, complete alloying and perfect adhesion of the alloy coating to the base metal. The coarsest and finest particles of powder are excluded but it is not essential that all of the particles shall be of the same size. Various mixtures which range in size from particles which will be retained on sieves about numbers 50 to 80 and will pass through sieves about numbers 16 to 30 may be used. Intermediate sizes may be used, for example powder which will pass through a number 30 sieve and will be retained on a number 60 sieve.

25 It is to be understood that alloy steels and irons may be used for the base metal as well as carbon steel, that variations in the thickness of the coatings of powder and binder and in the grading of the sizes of the particles may be made to vary the thickness and character of the alloy coatings, and that the content of chromium and iron may be varied within wide limits without departing from the invention.

35 The term, mold, as used in the specification and claims refers to the matrix which is used to give shape to the casting and may include the core as well as the parts of the mold which constitute the receptacle. The 40 sieve numbers in the specification and claims refer to the U. S. standard sieve numbers adopted by the American Society for Testing Materials.

I claim:—

45 1. A coating for molds adapted to form a chromium-containing alloy surface on a ferrous alloy base metal cast in the mold, which comprises a ferrochromium powder containing about 1% to 6% carbon and about 3% to 50 7% silicon.

55 2. A coating for molds adapted to form a chromium-containing alloy surface on a ferrous alloy base metal cast in the mold, which comprises a chromium alloy powder containing about 60.0% to 96.0% chromium, about 1% to 6% carbon and about 3% to 7% silicon.

60 3. A coating for molds adapted to form a chromium-containing alloy surface on a ferrous alloy base metal cast in the mold, which comprises a layer of metal powder about one thirty-second to one-eighth of an inch in thickness, said powder containing about 60% to 96% chromium, about 1% to 6% carbon, and about 3% to 7% silicon.

65 4. A coating for molds adapted to form a

chromium-containing alloy surface on a ferrous alloy base metal cast in the mold, which comprises a metal powder containing ferrochromium carrying about 1% to 6% carbon and about 60% to 95% chromium, and sufficient ferrosilicon to bring the silicon content of the powder to about 3% to 7%.

In testimony whereof, I affix my signature.

STANLEY M. NORWOOD.

70

75

80

85

90

95

100

105

110

115

120

125

130